# EUROPEAN PATENT APPLICATION

(11) **EP 0 254 781 A1**
(43) Date of publication of application: **03.02.1988**
(21) Application number: 86305801.2
(22) Date of filing: 29.07.1986
(51) Int. Cl.: C10G 25/00, C10G 61/06

(54) **Method of removing sulfur from a hydrocarbon feedstream**

(71) Applicant: CHEVRON RESEARCH COMPANY, San Francisco California 94120 (US)
(72) Inventor: Field, Leslie A., Oakland, CA 94618 (US)
(74) Representative: Kosmin, Gerald Emmanuel

(57) **Abstract**

Sulfur is removed from a hydrocarbon feedstream to a catalytic reformer by contacting the feedstream with a sulfur sorbent comprising a metal component containing a metal selected from Group I-A or Group II-A of the Periodic Table supported on a porous refractory inorganic oxide support.

## Description

This invention relates to a method of removing sulfur compounds from the hydrocarbon feedstreams to a catalytic reformer.

Catalytic reforming processes play an integral role in upgrading naphtha feedstocks to high octane gasoline blend stocks. These processes have become more important in recent years because of the increase in demand for low-lead and unleaded gasolines.

In typical modern reforming processes, the naphtha feed is passed over a promoted noble metal catalyst at a temperature in the range of 3l5°C to 595°C, a pressure in the range of from l atmosphere to 70 atmospheres, a liquid hourly space velocity (LHSV) in the range of .l to l0, and a hydrogen to hydrocarbon mole ratio in the range of l to l0. Variations in these conditions will depend in large measure upon the type of feed processed and the desired product octane level.

It is generally recognized that the sulfur content of the feedstock must be minimized to prevent poisoning of the reforming catalyst. Preferably, the feed will contain less than 2 to 5 parts per million by weight (ppm) of sulfur, since the presence of sulfur in the feed decreases both the activity and the selectivity of the catalyst. Certain reforming catalysts are extremely sulfur sensitive, and sulfur levels in the feed of even less than l ppm can severely deactivate these catalysts.

Sulfur sorbents can remove nearly all of the sulfur present in the feed at the high temperatures used in reforming. One sulfur sorbent that is used at low temperatures is a metal or metal compound, such as copper, which is supported on a porous refractory inorganic oxide support or on a carbon support. An example of such a sorbent is disclosed in U.S. Patent No. 4,204,947. That sorbent is copper supported on alumina. Other similar sorbents are disclosed in U.S. Patent Nos. 2,593,464 and 4,224,l9l. Copper on alumina works well as a sorbent for H₂S or mercaptan type sulfur, but copper sorbents tend to be less effective at higher temperatures, removing less sulfur as the temperature goes above 300°C. Furthermore, copper sorbents do not work on some types of sulfur which can be present in the reforming feed, such as thiophenic sulfur. Also, copper is costly.

Various promoter metals have been used in conjunction with copper. For example, U.S. Patent No. 4,008,l74 discloses copper and chromium on a carbon support. The chromium aids in regeneration of the sorbent.

The present invention is a novel method of removing sulfur from hydrocarbon feedstreams by using a metal component containing a metal selected from Group I-A or Group II-A of the Periodic Table supported on a porous refractory inorganic oxide support. Preferred metal components include sodium, potassium, calcium and barium. Preferred refractory inorganic oxide supports include alumina, silica, boria, titania, zirconia, aluminosilicates, aluminophosphates, and mixtures of two or more thereof.

One preferred method of making these sulfur sorbents is by impregnating a preformed porous refractory inorganic oxide support with an aqueous solution of a metal salt, where the metal is selected from Groups I-A or II-A of the Periodic Table, and drying and calcining the resulting material.

An alternative method is by peptizing a refractory inorganic oxide support, thereby forming a plastic mass, mulling the mass with a compound containing a Group I-A or Group II-A metal, then extruding the mass, and drying and calcining it.

For a better understanding of the invention, reference will now be made, by way of example, to the accompanying drawing which is a plot of the average catalyst temperature of an exemplary material required to maintain the target refractive index of the C₅+ liquid product of 1.4300, which corresponds to about 47 wt% aromatics in the feed.

A refinery produces naphtha fractions having substantial amounts of sulfur in the form of organic sulfides, such as thiophenes and mercaptans. Sometimes the sulfur level is higher than l00 ppm in the untreated naphtha fraction. These feeds with very high sulfur levels can be contacted with hydroprocessing catalysts to convert the sulfur compounds to H₂S. If the remaining sulfur level is too high, then the high sulfur level can cause the reforming catalyst to rapidly lose both activity and selectivity when used for reforming. Prudent operation demands that heavily sulfur contaminated feeds be further treated before contacting sulfur sensitive catalysts.

Preferred supports for the sulfur sorbent include alumina, silica, titania, zirconia, boria, and the like, and mixtures thereof. Clays can also be used as supports. Particular clays of interest include the fibrous magnesium silicate clays, for example, attapulgite, halloysite, palygorskite and sepiolite. The support can be premade by any method known in the art.

The surface area of the finished sulfur sorbent is in large part due to the support chosen. It is believed that the active sulfur sorbents of this invention can have nitrogen surface areas in the range of between 20 and 300 m₂/g.

Since the sulfur sorbents of this invention can be used for removing sulfur from feedstreams for reforming units, one typical feedstock will be low molecular weight hydrocarbons which are in the vapor phase at reforming conditions. In particular, the feedstock will normally comprise alkanes and naphthenic compounds having between about five and twelve carbon atoms. Hydrogen may also be present, such as the recycle hydrogen stream of a reforming unit. Because vapors diffuse rapidly into the pores of the support material, the precise size and pore distributions are not thought to be critical in a sulfur sorbent for use in this application.

The metal components of the sulfur sorbents in this invention can be Group I-A or Group II-A metal containing compounds. The preferred metal components are sodium, potassium, calcium, and barium. The metal components are not in general present as the reduced metal. Instead, they are usually present in the form of a salt, oxide, hydroxide, nitrate, or other compound. It is the metal in the compound, in any form, that is the metal component of the sorbent of this invention. The sulfur sorbents of this invention can be made by impregnation of a preformed refractory inorganic oxide support with a metal component, or by comulling the metal component with the inorganic oxide support.

Preferred metal compounds include sodium chloride, sodium nitrate, sodium hydroxide, sodium carbonate, sodium oxalate, potassium chloride, potassium nitrate, potassium carbonate, potassium oxalate, potassium hydroxide, barium chloride, barium nitrate, barium carbonate, barium oxalate, barium hydroxide, calcium chloride, calcium nitrate, calcium carbonate, calcium oxalate, calcium hydroxide, and the like.

A preformed inorganic support can be impregnated with Group I-A or Group II-A metals by standard techniques. It may be necessary to impregnate the support several times to achieve the desired amount of metal component on the inorganic support. Various metal compounds can be dissolved to form aqueous solutions useful for this impregnation. The preferred compounds for impregnation are the more soluble compounds. To be useful for impregnation, a compound should have a solubility of at least 0.l mole per liter of water.

Another method of making the sulfur sorbents of this invention is by mulling the powdered inorganic support material, which may be prepeptized or mixed in the presence of a peptizing agent, together with a compound containing a Group I-A or Group II-A metal. Preferred peptizing agents are mineral acids, such as nitric acid. For example, peptized alumina powder could be mixed with a metal component, such as potassium carbonate. The resulting mass is then extruded, dried and calcined to form the final sulfur sorbent.

The choice of the appropriate compound to use during fabrication of the sulfur sorbent is primarily dictated by the solubility of the salt. For example, in impregnation, very soluble salts are desired such as nitrates, but in mulling, relatively insoluble salts such as carbonates are preferred.

If sulfur is present that is not in the form of H₂S, it is preferred that the sulfur sorbent of this invention include being commingled with or preferably preceded by small amounts of platinum or palladium, either on the sorbent or on a suitable support. Between 0.0l weight percent and 0.5 weight percent platinum or palladium may be added. In the presence of added hydrogen, the added metals catalyze the conversion thiophenic and other organic type sulfur compounds that may exist in the feedstream into easily sorbed sulfur compounds. If the platinum or palladium is on the sorbent particles themselves, it may also reduce coking of the feed on the sorbent particles. When thiophenic and other organic sulfur compounds contact platinum and palladium, hydrogen sulfide is formed, which is readily removed by the sulfur sorbent.

The sorbent of this invention is used to remove sulfur from feedstocks containing sulfur levels as high as several percent to levels as low as l ppm (part per million) and lower. Typically, the sorbent and reforming catalyst are contained in separate vessels. The vessel containing the sulfur sorbent is typically placed upstream of the vessel containing the reforming catalyst. The feedstock may be heated to as high as the reforming reaction temperature or to a lower temperature before it contacts the sulfur sorbent; from ambient temperature to as high as l000°F (540°C) and higher.

The sorbent can be placed in the same reaction vessel as the reforming catalyst. If the sorbent is given the proper porosity and shape it can be inter-mixed with the reforming catalyst, in the same bed. As any residual organic sulfur is converted by the reforming catalyst to H₂S, the sorbent removes it, preventing harm to subsequent beds, and prolonging operational life of the system because the sorbent functions well at reforming temperatures.

The sorbent can safely contact the amounts of water normally found in reforming feedstreams. The feedstreams do not have to be as extraordinarily dry as they would if they were contacting the reduced, metallic form of alkali metals or alkaline earth metals and if this reduced, metallic form were required. Group I-A and Group II-A metals can form hydroxides or oxides in a water-containing stream. However, the water level in the hydrogen recycle stream should be kept low, preferably to less than l00 ppm, and more preferably to less than 50 ppm.

This sorbent can be used in combination with other sorbents. For instance, in one embodiment, the hydrocarbon feedstock is contacted with a hydrotreating catalyst to convert organic sulfur compounds in the feedstock, then the feedstock is contacted with a sorbent, such as zinc oxide or copper oxide, supported on a clay base, then the feedstock is contacted with the sorbent of the present invention.

In the following non-limitative examples, the preformed gamma alumina base used was a commercially available 1/16th inch (1.6 mm) extrudate, with a H₂O pore volume of approximately .7 cc/gm and a N₂ surface area of approximately 200 m²/gm. It was calcined at l250°F (677°C). It was made by peptizing a pseudoboehmite alumina of crystal size in the range of approximately 33 to 40 Angstroms as determined by X-ray diffraction (XRD) with an aqueous solution of a mineral acid, mixing it until it reached an extrudable state, then extruding, drying and calcining the resulting material.

### Example I

This example shows a sulfur sorbent of this invention. The sorbent was prepared by taking l00 gm of pre-extruded alumina and impregnating it with 25.9 gm KNO₃ in 76 ml H₂O, by pore fill impregnation. The sorbent was dried for l6 hours at 250°F (121°C) and then calcined for 2 hours at ll00°F (593°C). .12 ml of a solution of .093 gm Pt/ml, where the form of Pt was H₂PtCl₆, in distilled water was then impregnated onto the support. It was dried for 48 hours at 250°F (121°C) and calcined for 2 hours at 500°F (260°C). This composition of matter will be identified as A.

### Example II

This example shows another sulfur sorbent of this invention. 200 grams of pre-extruded alumina were impregnated with .22 ml of .093 gm Pt/ml, where the form of Pt was H₂PtCl₆, in l64 ml H₂O, under 30 inches (76.2 cm) of vacuum. The extrudate was then impregnated with 57.43 grams of potassium nitrate in l64 ml of water. The extrudate was dried at 250°F (121°C) overnight and then calcined for 2 hours at ll00°F (593°C). This composition of matter will be identified as B.

### Example III

This example shows the manufacture of a monometallic reforming catalyst. 50 grams of pre-extruded alumina was impregnated under 30 inches (76.2 cm) of vacuum with l.6 ml of an aqueous solution of H₂PtCl₆ of concentration .093 gm Pt/ml in 30 ml of H₂O. The impregnated alumina was allowed to stand for 2 hours and then dried at 250°F (121°C) overnight and then calcined for 2 hours at 950°F (510°C) in air. The catalyst produced can be used for reforming. This composition of matter will be identified as C.

### Example IV

l000 gm of an L zeolite of crystal size between l000 and 2000 Angstroms was mixed with l0 liters of .3 molar Ba(NO₃)₂ solution. The zeolite and solution were placed into 2 bottles. Lids were placed on the bottles and they were shaken. They were then placed into a preheated oven at 80°C for 3 hours. Then the contents were filtered and washed with 2 liters distilled water. The solids were dried for l6 hours at 250°F (121°C) and calcined for 16 hours at 1100°F (593°C) in air.

752.4 gm of smaller than l4 mesh powder made as above was impregnated with a solution of Pt(NH₃)₄(NO₃)₂ to 8 wt % Pt, in 752.4 ml of aqueous solution. This was then dried for l6 hours at 250°F (121°C), rescreened to < 14 mesh, and calcined for 2 hours at 500°F (260°C) in air. This composition of matter will be identified as D.

### Example V

This example was a standard reforming run using a sulfur-sensitive reforming catalyst except that (l) there was no sulfur sorber; and (2) l ppm sulfur was added to the feed after 480 hours. The catalyst in this example was D. The results before and after sulfur addition are shown in the following table. After 600 hours, control of temperature to maintain the required aromatics content was no longer possible due to rapid catalyst deactivation. After 670 hours, the addition of sulfur to the feed was discontinued, and clean feed was used. No recovery of activity was observed during 50 hours of clean feed operation. In addition, the feed was withdrawn at 720 hours, and the catalyst was stripped with sulfur-free hydrogen gas for 72 hours at 930°F (499°C). Only a small gain in activity was observed.

### Example VI

This example was run as shown in Example V, except that .5 ppm mercaptan-type sulfur was added to the feed from 270 hours to 360 hours on stream, and again from 455 hours to 505 hours on stream. After 450 hours, control of temperature to maintain the required aromatics content was no longer possible due to rapid catalyst deactivation. The results are shown below:

### Example VII

Deionized water was added to 0.23 ml of a solution containing 0.093 gm Pt/ml, the Pt as H₂PtC₁₆. The water was added until the total volume of the solution was l70 ml. This mixture was used to vacuum impregnate 200 gm of a preformed alumina extrudate. The impregnated extrudate was then allowed to stand for 2 hours at room temperature, and was then dried for l6 hours at 250°F (121°C).

Next, 294.6 gm of Ca(NO₃)2:4H20 was mixed into l00 ml hot deionized water, and stirred until clear. The solution was then evaporated, cooled, and the volume adjusted to l70 ml. This solution was then used to impregnate the extrudate under vacuum. The extrudate then sat for 2 hours at room temperature, and was then dried at 250°F (121°C) overnight.

Finally, the material was calcined at 1100°F (593°C) in flowing air.

This material will be designated E.

### Example VIII

To 3.2 ml of a solution of 0.093 gm Pt/ml, the Pt as H₂PtC₁₆, was added deionized water until the total solution volume reached 80 ml. This solution was then used to impregnate l00 gms of a preformed alumina extrudate under vacuum. The extrudate was allowed to sit for 2 hours at room temperature and was then dried for l6 hours at 250°F (121°C). Finally, it was calcined for 2 hours in flowing air at 950°F (510°C).

This material will be designated F.

### Example IX

To 1100 gm of an L zeolite was added 11 litres of an aqueous solution of 0.3 molar Ba as Ba(NO₃)₂. This mixture was placed in polypropylene bottles, the lids were closed, and the bottles were placed in a preheated 176°F(80°C).

After 4 hours, the contents of the bottles were poured off into filters and the solids collected. The filter solids were reslurried in fresh deionized water and refiltered to a total of 10 times.

The solids were then dried at 250°F (121°C) over a weekend, and calcined for 16 hours at 1100°F (593°C) in flowing air.

863.1 gm of the material was then screened to below l4 mesh. 0.8% Pt was added to the solids in a pore fill impregnation, using Pt(NH₃)₄(NO₃)₂ as the Pt source, and 690.5 ml of total solution. The material was allowed to sit at room temperature for 2 hours and was then dried at 250°F (121°C) for 16 hours.

Finally, the material was treated at 500°F (260°C) hours in flowing air.

This material will be designated G.

### Example X

This example shows the process of this invention. In a fixed bed tubular reactor, 25 cc of material F at 24 to 80 mesh was layered over 25 cc of material E at 24 to 80 mesh. This material was layered over l00 cc of material G, also at 24 to 80 mesh.

A naphtha feedstock of API gravity 67.0, boiling range as determined by D-86 distillation of start, 160°F (71°C ; 5% Pt. 167 (75); 10% Pt. 169 (76); 20% Pt. 171 (77); 30% Pt. 173 (78); 40% Pt. 175 (79); 50% Pt. 177 (81); 60% Pt. 180 (82); 70% Pt. 183 (84); 80% Pt. 190 (88); 90% Pt. 208 (98); 95% Pt. 208 (98); and end Pt. 254°F (123°C), and molecular type as determined by GC of 59.6 LV% paraffins, 36.6 LV% naphthenes, and 3.8 LV% aromatics, was fed over the catalyst at a l.5 LHSV relative to the reforming catalyst, N, at a pressure of l50 psig (l0 bar) and an H₂/HC ratio of 2. Organic sulfur as thiophene was doped into the feed and fed at a l to 2.5 ppm S level, based on feed.

Figure l is a plot of the catalyst average temperature of the material G required to maintain the target refractive index of the C₅+ liquid product of l.4300, which corresponds to about 47 wt% aromatics in the liquid.

The Pt containing material F in front of the sorbent material E serves to convert the thiophenic sulfur to H₂S, a form readily sorbed by the material.

Note that the reforming catalyst G was not deactivated by the sulfur to any measurable extent. Sulfur analyses on various layers of the catalysts after the completion of the run showed 440 and 370 ppm of sulfur on the Pt containing thiophene conversion catalyst F, l.27% S and l250 ppm S on the sorbent E, and 40, 24, and l8 ppm S on the reforming catalyst G.

## Claims

1. A method of removing sulfur from a hydrocarbon feedstream, which comprises contacting said hydrocarbon feedstream with a sulfur sorbent comprising a metal component containing a metal selected from Group I-A or Group II-A of the Periodic Table supported on a porous refractory inorganic oxide support.

2. A method according to Claim 1, wherein said metal component contains sodium, potassium, barium or calcium.

3. A method according to Claim 1 or 2, wherein said porous refractory inorganic oxide support is alumina, silica, zirconia, titania, boria, or a mixture of two or more thereof.

4. A method according to Claim 1 or 2, wherein said porous refractory inorganic oxide support is a clay selected from attapulgite, halloysite, palygorskite, and sepiolite.

5. A method according to Claim 1, 2, 3 or 4, wherein the hydrocarbon feedstream is contacted with a platinum or palladium conversion catalyst in addition to the sulfur sorbent,the location of the conversion catalyst being separate from or the same as the sulfur sorbent.

6. A method according to Claim 5, wherein the contacting of the hydrocarbon feedstream by the conversion catalyst precedes the contacting with the sulfur sorbent.

7. A method according to Claim 5, wherein the conversion catalyst and sulfur sorbent are used in the same reaction zone.

8. A method according to Claim 7, wherein the conversion catalyst and sulfur sorbent are inter-mixed.

9. A method according to any preceding claim, wherein the sulfur sorbent is prepared by:
(a) impregnating a preformed porous refractory inorganic oxide support with a solution comprising a solvent and a metal component containing a Group I-A or Group II-A metal of the Periodic Table; and
(b) drying and calcining the resulting impregnated material.

10. A method according to Claim 9, wherein said solution is an aqueous solution.

11. A method according to Claim 9 or 10, wherein said metal component has a solubility in water of at least 0.1 mole per liter of water.

12. A method according to any one of Claims 1 to 8, wherein the sulfur sorbent is prepared by:
(a) contacting the porous refractory inorganic oxide support and metal component to form an extrudable mass;
(b) mulling the extrudable mass;
(c) extruding the extrudable mass to form extrudates; and
(d) drying and calcining the extrudates to form the required sulfur sorbent.
